

March 31, 1953

2,633,241

M. K. BANKS  
FROTH FLOTATION OF IRON-BEARING  
MINERALS FROM FELDSPATHIC ORES  
Filed Feb. 1, 1951



*Mason K. Banks INVENTOR.*

*BY Bentley C. Morrow  
Attorney*

## UNITED STATES PATENT OFFICE

2,633,241

FROTH FLOTATION OF IRON-BEARING MIN-  
ERALS FROM FELDSPATHIC ORESMason K. Banks, Asheville, N. C., assignor to  
Tennessee Valley Authority, a corporation of  
the United States

Application February 1, 1951, Serial No. 208,948

9 Claims. (Cl. 209—166)

(Granted under Title 35, U. S. Code (1952),  
sec. 266)

## 1

The invention herein described may be manufactured and used by or for the Government for governmental purposes without payment to me of any royalty thereon.

This invention relates to the beneficiation of feldspathic ores. It concerns particularly the removal of iron-bearing minerals from such ores by froth flotation.

Feldspar for use in the glass trade must contain not more than 0.1 per cent iron, as  $Fe_2O_3$ , not more than 69 per cent silica, and not less than 18.0 per cent alumina. Size specifications require that the feldspar contain not more than 3 per cent of plus 20-mesh material and not more than 15 per cent of minus 200-mesh material.

Feldspar for use in the ceramic trade is ground to pass a 200-mesh screen. The alumina content usually should not be less than 18 per cent, although a few manufacturers place this requirement as low as 17 per cent. The principal requirement as to iron content is removal of all particles which might cause spotting or discoloring of fired ware. There is no definite specification on iron content except that spotting or discoloring due to iron must not occur when ceramic ware is fired. However, there is usually a close relationship between spotting and iron content of feldspar recovered as a flotation concentrate. Iron, expressed as  $Fe_2O_3$ , usually must be less than 0.05 per cent if spotting is to be avoided, and often should be around 0.03 per cent.

It is a general practice to recover feldspar from feldspathic ores as a flotation concentrate at minus 20 mesh. If produced for the glass market, the concentrate is then dried and shipped. If produced for the ceramic market, the concentrate is dried, is sometimes blended with block spar, ground to minus 200 mesh, sized, and shipped.

Large deposits of alaskite, a feldspathic ore, exist in western North Carolina. This material is a pegmatitic granite, varying in texture from the coarseness of pegmatite to the fineness of granite. It is rather uniform in composition, comprising oligoclase, quartz, microcline, and muscovite, with small amounts of garnet and biotite present, especially near the contacts.

Oligoclase is a soda-lime feldspar, and microcline is a potash feldspar. Muscovite and biotite are micaceous minerals. Biotite contains iron in its molecule. Muscovite, while it contains no iron

in its molecule, is frequently stained red or black by thin films of iron oxide between the laminae. Iron-containing garnets probably are present as almandite ( $3FeO \cdot Al_2O_3 \cdot 2SiO_2$ ) and/or andradite ( $3CaO \cdot Fe_2O_3 \cdot 3SiO_2$ ).

An alaskite ore sample, typical of that now being used in the production of feldspar in western North Carolina, had the following chemical analysis:

|                                | Per cent |
|--------------------------------|----------|
| SiO <sub>2</sub>               | 73.58    |
| Al <sub>2</sub> O <sub>3</sub> | 15.84    |
| Fe <sub>2</sub> O <sub>3</sub> | 0.43     |
| CaO                            | 1.08     |
| 15 Na <sub>2</sub> O           | 4.36     |
| K <sub>2</sub> O               | 4.10     |
| Ignition loss                  | 0.34     |
| Total                          |          |
|                                | 99.73    |

20 U. S. Patent No. 2,483,192 discloses a process for decreasing the ferrous-metals silicates content of feldspathic ore by pulping the ore with water, conditioning the pulped ore in an acid medium at a pH of 2.5 to 5.0 with a sulfonated petroleum hydrocarbon promoter with or without fuel oil and a suitable frother, subjecting the conditioned pulp to froth flotation, and removing the froth flotation concentrate. Since alaskite and certain other feldspathic ores contain both micaceous materials and garnets, known to require, respectively, a cationic and an anionic promoter for flotation, it might be expected that such process would be ineffective for producing ceramic-grade feldspar by simultaneous removal of iron-bearing impurities of both types. Laboratory tests reported in Example I, below, and plant experience have tended to confirm this assumption.

40 A process now in use for the removal of iron-bearing impurities from feldspathic ores containing iron both as micaceous materials and as garnets requires two flotation steps for iron removal. In the first step, the ground, screened, and deslimed ore is conditioned at about 50 per cent solids with appropriate amounts of sulfuric acid, fuel oil, a cationic promoter, usually a long-chain fatty-acid amine, and a suitable frother, usually a crude or refined pine oil. The conditioned pulp is then diluted and subjected to froth flotation, and a flotation concentrate consisting mainly of micaceous impurities is removed.

In the second step, the resulting flotation tailing is partially dewatered in a hydraulic classifier and then conditioned at about 65 per cent solids with appropriate amounts of fuel oil, sulfuric acid, an anionic promoter, which may be a sulfonated petroleum hydrocarbon, and a suitable frother. The conditioned pulp is then subjected to froth flotation, and the flotation concentrate, consisting mainly of garnet impurities, is removed. This process has proved successful for the production of ceramic-grade feldspar from such ores but, since two separate flotation steps are required to reduce the iron content to sufficiently low value, it is necessarily complicated and requires equipment, reagent, and handling expense exceeding that of a one-step process.

The prior art, however, as typified by U. S. Patent No. 2,483,192, column 4, lines 74-75 ff., and by an article entitled "Flotation—chemicals for non-metallic minerals," Rock Products 49, 88-93+, December 1946, has taught that cationic and anionic flotation promoters cannot be used together in a single step because they are antagonistic to each other and require different conditions for effectiveness.

It is an object of this invention to provide a one-step flotation process for the removal of iron from feldspathic ores containing iron both as micaceous materials and as garnets.

Another object is to provide a method for the production of ceramic-grade feldspar from feldspathic ores containing both micaceous materials and garnets.

Other objects and advantages will become apparent as this disclosure proceeds.

I have found that these objects may be attained by simultaneously conditioning a suitably ground and deslimed pulp of feldspathic ore containing iron both as micaceous materials and as garnets with suitable amounts of a cationic promoter comprising a long-chain fatty-acid amine and with an effective amount of an anionic promoter, namely, a material selected from the group consisting of sulfonated oleic acid, sulfonated red oil, sulfonated methyl esters of red oil, and Turkey red oil, in an acid medium, with or without suitable frothing and/or oiling agents; subjecting the conditioned pulp to froth flotation; and removing the iron-bearing minerals in froth as a flotation concentrate. A flotation-cell tailing consisting essentially of feldspar and quartz is then withdrawn and is conditioned with hydrofluoric acid and a long-chain fatty-acid amine—preferably the same amine used in floating the iron-bearing minerals—with or without suitable frothing and/or oiling agents. This pulp is then subjected to froth flotation, and feldspar sufficiently free from iron to pass specifications for ceramic-grade material is recovered as a flotation concentrate.

The drawing submitted herewith is a diagrammatic flowsheet of a process embodying principles of my invention. Steps which are novel in themselves are indicated by solid lines, and other steps which may be necessary in the process but which are, in themselves, old in the art are indicated by broken lines.

Reference to this flowsheet shows that alaskite or other feldspathic ore containing iron both as micaceous materials and as garnets is fed into a crusher. A jaw crusher usually is used for the purpose of reducing the lumps of ore to such sizes as can be efficiently handled by a grinding mill. A suitable quantity of wa-

ter is added to the crushed ore and it is passed to a grinding mill, preferably a rod mill, where the ore is ground to pass a 20-mesh screen. The ground ore is passed to a suitable means for removing 20-mesh oversize material, preferably a 20-mesh screen, and any oversize is removed. That fraction of the ground ore of sizes passing the 20-mesh screen is then advanced to a means for removing slimes, preferably a hydraulic classifier, and substantially all minus 325-mesh material is separated from the bulk of the ore. The steps just described are old in the art and are preferred merely because of cheapness or convenience. Any equivalents therefor may be substituted if desired, as it is merely necessary that the ore be reduced to particles of such size as to pass a 20-mesh screen, and that minus 325-mesh slimes be removed.

A pulp of the resulting ground, deslimed ore containing about 55 per cent to 65 per cent solids is introduced into a conditioner. Sulfuric or other acid or acid salt yielding a free acidic radical in solution is added in quantity sufficient to maintain the pulp in the pH range from about 2.0 to 3.6 and preferably in the range from about 2.0 to 3.1. I have found that iron removal is satisfactory up to pH 3.6 and above, but above 3.6 excessive quantities of feldspar and quartz will be floated with the iron-bearing minerals. A material selected from the group consisting of sulfonated oleic acid, sulfonated red oil, sulfonated methyl esters of red oil, and Turkey red oil, is added as anionic-flotation promoter, and a long-chain fatty-acid amine or mixture of such amines or water-soluble salts of such amines yielding the amines in solution is also added to serve as cationic-flotation promoter. A frothing agent such as pine oil may be required when certain sulfonated fatty acid materials are used, and is also added if necessary. An oiling agent such as fuel oil also may be added if desired.

The resulting conditioned pulp is then passed to a flotation cell and is adjusted to a concentration of about 25 per cent solids by the addition of water. The resulting pulp is subjected to froth flotation, and iron-bearing minerals of both micaceous and garnet types are removed in froth as a flotation concentrate.

The amount of each class of promoter required to be added in the conditioning step described above will depend on a number of factors, but mainly on the amount of iron-bearing minerals to be removed from the ore and on the degree of purity of reagents employed. In general, about 0.5 to 2.0 pounds of sulfonated fatty acid, acids, or fatty-acid esters and about 0.1 to 0.5 pound of long-chain fatty-acid amine or amines will be required per ton of ore treated.

As used in this specification, the term "long-chain sulfonated fatty acid" refers to compounds having 14 or more carbon atoms in the fatty-acid radical, and since the sulfate group often is present to some extent in commercial sulfonated fatty acids the term is not intended to exclude the presence of acids having the sulfate group present as such. The term "long-chain fatty-acid amine" refers to such amines having 14 or more carbon atoms in the fatty-acid radical.

I have found that in the presence of feldspathic ore and under the conditions described certain anionic promoters comprising a sul-

sulfonated long-chain fatty acid, namely, a material selected from the group consisting of sulfonated oleic acid, sulfonated red oil, sulfonated methyl esters of red oil, and Turkey red oil, are not antagonistic to cationic promoters comprising a long-chain fatty-acid amine, but each exerts its full selective flotation effect under identical conditions. These promoters may therefore be used together in a single flotation step. The expected antagonism is not detectable, although other anionic promoters such as sulfonated petroleum oils and many sulfonated long-chain fatty-acid materials are antagonistic to long-chain fatty-acid amines under similar conditions.

After removal of iron-bearing minerals by flotation, the resulting flotation tailing is passed to a means for removing water, preferably a hydraulic classifier. It is there concentrated to about 50 per cent solids by removing water and is passed to a second conditioner. The pulp is there conditioned with suitable amounts of hydrofluoric acid, a long-chain fatty-acid amine (preferably the same used in the iron-removal step described above), a suitable frothing agent, and fuel oil. The resulting conditioned pulp is diluted with water if necessary and is then subjected to froth flotation. Feldspar sufficiently low in iron for use in the ceramic trade is thereby recovered in froth as a flotation concentrate.

Examples are given below illustrating quantities of reagents and conditions which have proved effective for the production of ceramic-grade feldspar from ores containing iron both as micaceous materials and as garnets. Other examples illustrate the failure of methods of the prior art to produce such results.

The Examples I through VII describe laboratory-scale batchwise tests. In each of these examples the following procedure was used in preparing the ore for testing:

- (a) A 600-gram sample of crushed ore was wet-ground at 25 per cent solids in a rod mill for 2 to 3 minutes.
- (b) The ground ore was passed through a 20-mesh screen, and the 20-mesh oversize was discarded.
- (c) The minus 20-mesh material was deslimed by washing three times on a 325-mesh screen.

The quantities of reagents given in all the following examples are in terms of pounds of reagents per ton of feed to the grinder.

Trade names are given for the reagents used, since pure compounds are seldom employed as flotation promoters, and it may be necessary to vary the amounts slightly if other approximately equivalent materials are substituted for those described. The materials identified by their trade names, are defined as follows:

- (a) "Ahcol 550" is a fairly pure sulfonated oleic acid.
- (b) "Ahcol 575" is crude sulfonated oleic acid and is sulfonated red oil.
- (c) "Ahcol 385" is a mixture of sulfonated oleic, linoleic, and rosin acids, prepared by sulfonating tall oil.
- (d) "RL-408" is a flotation reagent prepared by esterifying red oil with methyl alcohol, distilling off the esters, and sulfonating the distillate by digesting with concentrated sulfuric acid.
- (e) Turkey red oil is a sulfonated and sulfated castor oil.

- (f) "Amine 22T" is a mixture of long-chain fatty-acid amines prepared from tall oil.
- (g) "Armac T" is a mixture of water-soluble acetate salts of hexadecyl, octadecyl, and octadecenyl amines prepared from tallow.
- (h) "Reagent 825" is a sulfonated petroleum hydrocarbon material of the oil-soluble, water-dispersible "mahogany" type.
- (i) "Aerofloat 31" is a frothing agent which comprises about 6 per cent thiocarbanilide dissolved in dicesyl dithio phosphoric acid.
- (j) "B-23" is a synthetic frother consisting essentially of higher alcohols.

#### EXAMPLE I.

The process of U. S. 2,483,192 was tested to determine its effectiveness with alaskite. The ore used in this test contained 0.41 per cent  $Fe_2O_3$ . The promoter used was "Reagent 825." The deslimed ore was conditioned for 6 minutes at 70 per cent solids with 0.35 lb./ton sulfuric acid, 1.2 lb./ton "Reagent 825," 0.25 lb./ton "Aerofloat 31," and 0.50 lb./ton of fuel oil. The pulp was diluted to flotation density (about 25 per cent solids), subjected to froth flotation, and the froth concentrate was separated.

Visual examination of the cell tailing, containing feldspar and quartz, showed that removal of the garnet impurities was good, but that removal of micaceous material was incomplete. The  $Fe_2O_3$  content of the cell tailing, as determined by chemical analysis, was 0.061 per cent.

The cell tailing was then conditioned at 55 per cent solids with 1.50 lb./ton hydrofluoric acid, 0.50 lb./ton fuel oil, 0.25 lb./ton "B-23," and 0.25 lb./ton "Armac T." The conditioned pulp was subjected to froth flotation, and the feldspar flotation concentrate was removed.

The results of the test are tabulated below:

Table I-A

|                      | Wt., gr. | Per cent, Wt. | Per cent, $Al_2O_3$ | Per cent, $Fe_2O_3$ | Per cent, $SiO_2$ |
|----------------------|----------|---------------|---------------------|---------------------|-------------------|
| Feed                 | 600      | 100.0         | -----               | 0.41                | -----             |
| Iron concentrate     | 36       | 6.0           | -----               | -----               | -----             |
| Feldspar concentrate | 339      | 56.5          | 19.6                | 0.067               | 66.6              |
| Quartz tail          | 135      | 23.5          | -----               | 0.048               | 96.9              |
| Loss <sup>1</sup>    | 90       | 15.0          | -----               | -----               | -----             |

<sup>1</sup> Loss represents plus 20-mesh material, and minus 325-mesh material.

The feldspar concentrate produced by this process met the specifications for glass-grade feldspar. The feldspar, however, contained numerous black particles of biotite, as well as clear mica, and would not have been suitable for use in high-grade ceramic ware.

#### EXAMPLE II

In another test, reagent "RL-408" was used instead of "Reagent 825" with the same ore used in Example I.

The deslimed ore was conditioned for 6 minutes at 70 per cent solids with 0.35 lb./ton sulfuric acid, 1.2 lb./ton "RL-408," and 0.5 lb./ton fuel oil. The pulp was subjected to froth flotation, and the froth was separated. Separation of garnets was good, but mica separation was very poor. The cell tailing contained 0.219 per cent  $Fe_2O_3$ .

The cell tailing was then conditioned with 1.5 lb./ton hydrofluoric acid, 0.5 lb./ton fuel oil, 0.25 lb./ton "B-23," and 0.14 lb./ton "Armac T," and subjected to froth flotation. Separation of feldspar from quartz was poor.

The results of this test are tabulated below:

Table 2-A

|                           | Wt., gr. | Per cent Wt. | Per cent Al <sub>2</sub> O <sub>3</sub> | Per cent Fe <sub>2</sub> O <sub>3</sub> | Per cent SiO <sub>2</sub> |
|---------------------------|----------|--------------|-----------------------------------------|-----------------------------------------|---------------------------|
| Feed.....                 | 600      | 100.0        | -----                                   | 0.41                                    | -----                     |
| Iron concentrate.....     | 10       | 1.7          | -----                                   | -----                                   | -----                     |
| Feldspar concentrate..... | 315      | 52.5         | 20.2                                    | 0.30                                    | 64.9                      |
| Quartz tail.....          | 198      | 33.0         | -----                                   | 0.091                                   | 89.7                      |
| Loss.....                 | 77       | 12.8         | -----                                   | -----                                   | -----                     |

The feldspar concentrate produced in this test did not meet specifications for either glass-grade material or ceramic-grade, because of high Fe<sub>2</sub>O<sub>3</sub> and micaceous impurities.

## EXAMPLE III

In this test, my preferred procedure was followed. Deslimed pulp was conditioned for 10 minutes at 60 per cent solids with 0.35 lb./ton sulfuric acid, 1.2 lb./ton "RL-408," 0.5 lb./ton fuel oil, and 0.32 lb./ton "Armac T." The conditioned pulp was subjected to froth flotation, and the iron-bearing froth was separated. Removal of both garnets and mica was very good. The cell tailing contained 0.0278 per cent Fe<sub>2</sub>O<sub>3</sub>.

The cell tailing was then conditioned at 55 per cent solids with 1.5 lb./ton hydrofluoric acid, 0.5 lb./ton fuel oil, 0.25 lb./ton "B-23," and 0.14 lb./ton "Armac T," and the conditioned pulp was subjected to froth flotation.

Results:

Table 3-A

|                           | Wt., gr. | Per cent Wt. | Per cent Al <sub>2</sub> O <sub>3</sub> | Per cent Fe <sub>2</sub> O <sub>3</sub> | Per cent SiO <sub>2</sub> |
|---------------------------|----------|--------------|-----------------------------------------|-----------------------------------------|---------------------------|
| Feed.....                 | 600      | 100.0        | -----                                   | 0.41                                    | -----                     |
| Iron concentrate.....     | 35       | 5.8          | -----                                   | -----                                   | -----                     |
| Feldspar concentrate..... | 358      | 59.7         | 19.5                                    | 0.032                                   | 66.8                      |
| Quartz tail.....          | 130      | 21.7         | -----                                   | 0.024                                   | 97.0                      |
| Loss.....                 | 77       | 12.8         | -----                                   | -----                                   | -----                     |

The feldspar concentrate met specifications for ceramic-grade feldspar in all respects. Moreover, the separation of feldspar from quartz in the final flotation step was highly selective, as evidenced by the high SiO<sub>2</sub> content (97%) of the quartz tail.

## EXAMPLE IV

In this test, the identical procedure followed

Separation of feldspar from quartz in the second flotation step was incomplete, and the feldspar concentrate contained much of the mica that had not been removed in the first flotation step.

Results:

Table 4-A

|                           | Wt., gr. | Per cent Wt. | Per cent Al <sub>2</sub> O <sub>3</sub> | Per cent Fe <sub>2</sub> O <sub>3</sub> | Per cent SiO <sub>2</sub> |
|---------------------------|----------|--------------|-----------------------------------------|-----------------------------------------|---------------------------|
| Feed.....                 | 600      | 100.0        | -----                                   | 0.41                                    | -----                     |
| Iron concentrate.....     | 24       | 4.0          | -----                                   | -----                                   | -----                     |
| Feldspar concentrate..... | 240      | 40.0         | 19.9                                    | 0.140                                   | 65.0                      |
| Quartz tail.....          | 245      | 40.8         | -----                                   | 0.081                                   | 85.0                      |
| Loss.....                 | 91       | 15.2         | -----                                   | -----                                   | -----                     |

## EXAMPLE V

The following Table 5-A gives the results of tests which show the iron-removal efficiency of various sulfonated fatty-acid reagents in combination with long-chain fatty-acid amines. Table 5-B gives the reagent combinations that were used in each of the tests reported in Table 5-A.

Results tabulated under test 5-b were obtained by the use of "Ahcol 385," prepared by sulfonating tall oil. These particular results were very good but were obtainable only when the ore was of such nature as to require restricted amounts of anionic and cationic promoters. When larger amounts of reagent were necessary, it was found that a definite antagonism existed between such sulfonated tall oil and long-chain fatty-acid amines.

In each of these tests conditioning of the deslimed ore was carried out at 55 per cent solids.

Table 5-A

| Test No.         | Percent Fe <sub>2</sub> O <sub>3</sub> in feed | Percent Wt. |       |      | Percent Fe <sub>2</sub> O <sub>3</sub> in tail | Percent of Fe <sub>2</sub> O <sub>3</sub> removed |
|------------------|------------------------------------------------|-------------|-------|------|------------------------------------------------|---------------------------------------------------|
|                  |                                                | Feed        | Conc. | Tail |                                                |                                                   |
| 45               | 0.48                                           | 100         | 11.0  | 79.0 | 0.067                                          | 89.0                                              |
| 5-a <sup>1</sup> | 0.51                                           | 100         | 8.0   | 77.5 | 0.063                                          | 90.4                                              |
| 5-b <sup>1</sup> | 0.44                                           | 100         | 10.7  | 78.0 | 0.080                                          | 86.0                                              |
| 5-c <sup>1</sup> | 0.43                                           | 100         | 9.7   | 78.3 | 0.040                                          | 92.7                                              |
| 5-d <sup>1</sup> | 0.41                                           | 100         | 12.8  | 76.0 | 0.065                                          | 88.1                                              |
| 5-e <sup>1</sup> | 0.41                                           | 100         | 12.8  | 76.0 | 0.065                                          | 88.1                                              |

<sup>1</sup> Preconditioned for 3 minutes with 2.0 lb./ton NaOH prior to desliming.

Table 5-B

| Test No. | Reagents-lb./ton               |                    |                   |              |          |
|----------|--------------------------------|--------------------|-------------------|--------------|----------|
|          | H <sub>2</sub> SO <sub>4</sub> | Anionic promoter   | Cationic promoter | Frother      | Fuel oil |
| 5-a      | 0.8                            | 2.0 Turkey red oil | 0.25 "Amine 22 T" | 0.5 pine oil | -----    |
| 5-b      | 0.6                            | 1.5 "Ahcol 385"    | 0.1 "Armac T"     | 0.3 pine oil | -----    |
| 5-c      | 0.5                            | 1.5 "Ahcol 550"    | 0.2 "Armac T"     | do           | -----    |
| 5-d      | 0.9                            | 1.0 "Ahcol 575"    | 0.3 "Armac T"     | -----        | -----    |
| 5-e      | 0.35                           | 1.0 "RL-408"       | 0.32 "Armac T"    | -----        | 0.5      |

in Example III was used, except that 1.2 lb./ton of "Reagent 825" was substituted for 1.2 lb./ton of "RL-408."

Removal of garnets in the first flotation step was very good, but mica removal was poor. Antagonism between the sulfonated petroleum oil "Reagent 825" and the amine "Armac T" was clearly shown. Simultaneous removal of mica and garnets was not obtained. The cell tailing contained 0.11 per cent Fe<sub>2</sub>O<sub>3</sub>.

## EXAMPLE VI

The following Table 6-A gives the results of tests in which the effect of pH on iron-removal efficiency was investigated. The alaskite ore used in these tests contained 0.43 per cent Fe<sub>2</sub>O<sub>3</sub>. In these tests the deslimed ore was conditioned for 10 minutes at 55 per cent solids with varied amounts of sulfuric acid, 0.85 lb./ton "RL-408," 0.5 lb./ton fuel oil, and 0.32 lb./ton "Armac T." Following conditioning, the pulp was subjected to froth flotation for 3 minutes at 25 per cent solids.

Table 6-A

| Test No. | Lb./ton H <sub>2</sub> SO <sub>4</sub> | pH measured in conditioner | Percent Wt. |       |      | Percent Fe <sub>2</sub> O <sub>3</sub> removed |      |
|----------|----------------------------------------|----------------------------|-------------|-------|------|------------------------------------------------|------|
|          |                                        |                            | Feed        | Conc. | Tail |                                                |      |
| 7-a      | 0.05                                   | 5.0                        | 100.0       | 35.0  | 53.3 | 0.033                                          | 96.0 |
| 7-b      | 0.10                                   | 4.6                        | 100.0       | 33.8  | 54.0 | 0.034                                          | 95.5 |
| 7-c      | 0.15                                   | 4.1                        | 100.0       | 28.3  | 59.8 | 0.047                                          | 93.5 |
| 7-d      | 0.20                                   | 3.6                        | 100.0       | 16.3  | 72.6 | 0.028                                          | 96.1 |
| 7-e      | 0.25                                   | 3.45                       | 100.0       | 12.0  | 76.3 | 0.031                                          | 94.5 |
| 7-f      | 0.30                                   | 3.1                        | 100.0       | 7.0   | 81.4 | 0.035                                          | 93.4 |
| 7-g      | 0.40                                   | 2.8                        | 100.0       | 5.8   | 82.4 | 0.036                                          | 93.1 |
| 7-h      | 0.50                                   | 2.7                        | 100.0       | 5.8   | 82.3 | 0.018                                          | 96.5 |
| 7-i      | 0.60                                   | 2.6                        | 100.0       | 6.0   | 82.3 | 0.044                                          | 91.6 |
| 7-j      | 0.80                                   | 2.4                        | 100.0       | 6.5   | 84.5 | 0.038                                          | 92.6 |
| 7-k      | 1.00                                   | 2.1                        | 100.0       | 4.7   | 84.0 | 0.033                                          | 93.5 |

Iron-removal efficiency in all these tests was good, and pH seemed to have no significant effect on iron removal. However, pH had a marked effect on the amount of feldspar and quartz that was floated along with the iron-bearing minerals. It will be noted that at pH above 3.6 the weight per cent of the froth concentrate increased greatly. Since this represents a loss of feldspar, it is best to operate at a pH below 3.6 in the conditioner (calculations show that the pH increases from 0.1 to 0.2 upon dilution of the pulp to flotation density), and preferably within the range of about 2.0 to 3.1.

## EXAMPLE VII

In order to demonstrate the applicability of my process to ores other than alaskite, tests were carried out on a pegmatite-type ore. This ore differed from alaskite in that the muscovite and biotite present were of types different from those occurring in alaskite, and in that segregated crystalline masses of feldspar and mica were larger. Also, the general texture of the ore was coarser than that of alaskite.

The results of one of the tests of this ore are given in Table 7-A. In these tests the ore was crushed, screened, and deslimed in the same manner as in the alaskite tests.

In the test given in Table 7-A, the deslimed pulp was conditioned for 10 minutes at 60 per cent solids with 0.3 lb./ton sulfuric acid, 1.1 lb./ton "RL-408," 0.5 lb./ton fuel oil, and 0.32 lb./ton "Armac T." Upon removal of the iron-bearing minerals by froth flotation, the feldspar-quartz tail contained 0.037 per cent Fe<sub>2</sub>O<sub>3</sub>.

Following the iron-removal flotation step, the feldspar-quartz pulp was conditioned for 6 minutes at 45 per cent solids with 1.5 lb./ton hydrofluoric acid, 0.5 lb./ton fuel oil, 0.25 lb./ton "B-23," and 0.30 lb./ton "Armac T." The pulp was then subjected to froth flotation.

## Results:

Table 7-A

|                      | Wt., gr. | Per cent Wt. | Per cent Al <sub>2</sub> O <sub>3</sub> | Per cent Fe <sub>2</sub> O <sub>3</sub> | Per cent SiO <sub>2</sub> |
|----------------------|----------|--------------|-----------------------------------------|-----------------------------------------|---------------------------|
| Feed                 | 600      | 100.0        | -----                                   | 0.44                                    | -----                     |
| Iron concentrate     | 52       | 10.3         | -----                                   | -----                                   | -----                     |
| Feldspar concentrate | 300      | 50.0         | 18.9                                    | 0.038                                   | 367.8                     |
| Quartz tail          | 156      | 26.0         | -----                                   | 0.036                                   | 98.3                      |
| Loss                 | 82       | 13.7         | -----                                   | -----                                   | -----                     |

The feldspar produced was suitable in all respects for ceramic use.

## EXAMPLE VIII

Several pilot-plant tests were conducted to demonstrate the continuous operation of my

process. The flow diagram of the pilot plant in which these tests were carried out was substantially the same as that shown in the attached drawing. The raw material tested was an alaskite ore that contained 0.41 per cent Fe<sub>2</sub>O<sub>3</sub>.

Table 8-A gives the results of one of these tests. Table 8-B gives the quantities of reagents used in that test. Table 8-C gives the retention time of material within some of the pilot-plant units.

Table 8-A

|                                               | Pounds solids per hr. | Percent Wt. | Percent Al <sub>2</sub> O <sub>3</sub> | Percent Fe <sub>2</sub> O <sub>3</sub> | Percent SiO <sub>2</sub> |
|-----------------------------------------------|-----------------------|-------------|----------------------------------------|----------------------------------------|--------------------------|
| Feed to grinding mill                         | 300                   | 100.0       | 15.75                                  | 0.41                                   | 73.96                    |
| 20-mesh screen oversize                       | 4.5                   | 1.5         | -----                                  | -----                                  | -----                    |
| No. 1 hydraulic classifier overflow           | 32.0                  | 10.7        | -----                                  | -----                                  | -----                    |
| No. 1 flotation cell concentrate <sup>1</sup> | 30.0                  | 10.0        | -----                                  | -----                                  | -----                    |
| No. 1 flotation cell tail <sup>2</sup>        | 224.5                 | 74.7        | -----                                  | 0.0224                                 | -----                    |
| No. 2 hydraulic classifier overflow           | 11.5                  | 10.5        | -----                                  | -----                                  | -----                    |
| No. 2 flotation cell concentrate <sup>3</sup> | 165.0                 | 55.0        | 18.8                                   | 0.024                                  | 68.0                     |
| No. 2 flotation cell tail <sup>4</sup>        | 158.0                 | 19.3        | -----                                  | 0.018                                  | 69.0                     |
| Unaccounted for                               | 9.0                   | 3.0         | -----                                  | -----                                  | -----                    |

<sup>1</sup> Iron-bearing minerals.

<sup>2</sup> Feldspar plus quartz.

<sup>3</sup> Feldspar.

<sup>4</sup> Quartz.

<sup>5</sup> Not included in totals.

Table 8-B

|                                          | Reagents          | Cubic centimeters per minute | Pounds per ton of feed |
|------------------------------------------|-------------------|------------------------------|------------------------|
| Iron-removal flotation step <sup>1</sup> | Sulfuric acid     | 22                           | 0.5                    |
|                                          | "RL-408"          | 25                           | 1.2                    |
|                                          | "Armac T"         | 14                           | 0.32                   |
|                                          | Fuel oil          | 1.2                          | 1.0                    |
| Feldspar flotation step:                 | Hydrofluoric acid | 3.0                          | 11.25                  |
|                                          | "Armac T"         | 8.0                          | 0.15                   |
|                                          | Fuel oil          | 0.6                          | 0.50                   |
|                                          | "B-23"            | 0.3                          | 0.25                   |

<sup>1</sup> pH in conditioner = 2.7.

Table 8-C

|                       | Unit  | Retention time, minutes |
|-----------------------|-------|-------------------------|
| First conditioner     | ----- | 10                      |
| First flotation cell  | ----- | 5                       |
| Second conditioner    | ----- | 4                       |
| Second flotation cell | ----- | 5                       |

As a result of the tests described in the above examples and of other experimental work, it was found that "RL-408" is exceptionally effective in my process; it is the preferred material for use as anionic promoter therein.

I claim as my invention:

1. A process for the production of ceramic-grade feldspar from a feldspathic ore containing iron both as micaceous materials and as garnets which comprises mixing such ore in a ground, deslimed state with water to form a pulp containing about 55 to 65 per cent solids, simultaneously conditioning the resulting pulp with a sufficient amount of a material selected from the group consisting of water-soluble acids and acid salts yielding free acidic radicals in solution to produce a pH of about 2.0 to 3.6 in the pulp, with an effective amount of an anionic promoter comprising a material selected from the group consisting of sulfonated oleic acid, sulfonated red oil, sulfonated methyl esters of red oil, and Turkey

red oil, and with an effective amount of a cationic promoter comprising a long-chain fatty-acid amine; diluting the resulting conditioned pulp with water to a concentration of about 25 per cent solids; subjecting the resulting diluted pulp to froth flotation; removing resulting froth containing both micaceous materials and garnets; removing water from the resulting flotation tailing to a concentration of about 50 per cent solids; conditioning the resulting concentrated tailing with effective amounts of hydrofluoric acid, a long-chain fatty-acid amine, and a frothing agent; subjecting the conditioned tailing to froth flotation; and recovering ceramic-grade feldspar in froth as a flotation concentrate.

2. A process for the production of ceramic-grade feldspar from a feldspathic ore containing iron both as micaceous materials and as garnets which comprises mixing such ore in a ground, deslimed state with water to form a pulp containing about 55 to 65 per cent solids; simultaneously conditioning the resulting pulp with a sufficient amount of a material selected from the group consisting of water-soluble acids and acid salts yielding free acidic radicals in solution to produce a pH of about 2.0 to 3.6 in the pulp, with an effective amount of an anionic promoter comprising sulfonated methyl esters of red oil, and with an effective amount of a cationic promoter comprising a long-chain fatty-acid amine; diluting the resulting conditioned pulp with water to a concentration of about 25 per cent solids; subjecting the resulting diluted pulp to froth flotation; removing resulting froth containing both micaceous materials and garnets; removing water from the resulting flotation tailing to a concentration of about 50 per cent solids; conditioning the resulting concentrated tailing with effective amounts of hydrofluoric acid, a long-chain fatty-acid amine, and a frothing agent; subjecting the conditioned tailing to froth flotation; and recovering ceramic-grade feldspar in froth as a flotation concentrate.

3. A process for the production of ceramic-grade feldspar from a feldspathic ore containing iron both as micaceous materials and as garnets which comprises mixing such ore in a ground, deslimed state with water to form a pulp containing about 55 to 65 per cent solids; simultaneously conditioning the resulting pulp with a sufficient amount of a material selected from the group consisting of water-soluble acids and acid salts yielding free acidic radicals in solution to produce a pH of about 2.0 to 3.6 in the pulp, with an effective amount of an anionic promoter comprising a material selected from the group consisting of sulfonated oleic acid, sulfonated red oil, sulfonated methyl esters of red oil, and Turkey red oil, and with an effective amount of a cationic promoter comprising a mixture of hexadecyl, octadecyl, and octadecenyl amines; diluting the resulting conditioned pulp with water to a concentration of about 25 per cent solids; subjecting the resulting diluted pulp to froth flotation; removing resulting froth containing both micaceous materials and garnets; removing water from the resulting flotation tailing to a concentration of about 50 per cent solids; conditioning the resulting concentrated tailing with effective amounts of hydrofluoric acid, a long-chain fatty-acid amine, and a frothing agent; subjecting the conditioned tailing to froth flotation; and recovering ceramic-grade feldspar in froth as a flotation concentrate.

4. A process for removing iron-bearing min-

erals from a feldspathic ore containing iron both as micaceous materials and as garnets which comprises pulping such ore as minus 20-mesh deslimed particles with water to form a pulp containing about 55 to 65 per cent solids; simultaneously conditioning the resulting pulp with a sufficient amount of a material selected from the group consisting of water-soluble acids and acid salts yielding free acidic radicals in a solution to produce a pH of about 2.0 to 3.6 in the pulp, with an effective amount of an anionic promoter comprising a material selected from the group consisting of sulfonated oleic acid, sulfonated red oil, sulfonated methyl esters of red oil, and Turkey red oil, and with an effective amount of a cationic promoter comprising a long-chain fatty-acid amine; diluting the resulting conditioned pulp with water to a concentration of about 25 per cent solids; subjecting the resulting diluted pulp to froth flotation; and removing the resulting froth containing both micaceous materials and garnets.

5. A process for removing iron-bearing mineral from a feldspathic ore containing iron both as micaceous materials and as garnets which comprises pulping such ore as minus 20-mesh deslimed particles with water to form a pulp containing about 55 to 65 per cent solids; simultaneously conditioning the resulting pulp with a sufficient amount of a material selected from the group consisting of water-soluble acids and acid salts yielding free acidic radicals in a solution to produce a pH of about 2.0 to 3.6 in the pulp, with an effective amount of an anionic promoter comprising sulfonated oleic acid, and with an effective amount of a cationic promoter comprising a long-chain fatty-acid amine; diluting the resulting conditioned pulp with water to a concentration of about 25 per cent solids; subjecting the resulting diluted pulp to froth flotation; and removing the resulting froth containing both micaceous materials and garnets.

6. A process for removing iron-bearing minerals from a feldspathic ore containing iron both as micaceous materials and as garnets which comprises pulping such ore as minus 20-mesh deslimed particles with water to form a pulp containing about 55 to 65 per cent solids; simultaneously conditioning the resulting pulp with a sufficient amount of a material selected from the group consisting of water-soluble acids and acid salts yielding free acidic radicals in a solution to produce a pH of about 2.0 to 3.6 in the pulp, with an effective amount of an anionic promoter comprising sulfonated red oil, and with an effective amount of a cationic promoter comprising a long-chain fatty-acid amine; diluting the resulting conditioned pulp with water to a concentration of about 25 per cent solids; subjecting the resulting diluted pulp to froth flotation; and removing the resulting froth containing both micaceous materials and garnets.

7. A process for removing iron-bearing minerals from a feldspathic ore containing iron both as micaceous materials and as garnets which comprises pulping such ore as minus 20-mesh deslimed particles with water to form a pulp containing about 55 to 65 per cent solids; simultaneously conditioning the resulting pulp with a sufficient amount of a material selected from the group consisting of water-soluble acids and acid salts yielding free acidic radicals in a solution to produce a pH of about 2.0 to 3.6 in the pulp, with an effective amount of an anionic promoter comprising sulfonated methyl esters of

red oil, and with an effective amount of a cationic promoter comprising a long-chain fatty-acid amine; diluting the resulting conditioned pulp with water to a concentration of about 25 per cent solids; subjecting the resulting diluted pulp to froth flotation; and removing the resulting froth containing both micaceous materials and garnets.

8. A process for removing iron-bearing minerals from a feldspathic ore containing iron both as micaceous materials and as garnets which comprises pulping such ore as minus 20-mesh deslimed particles with water to form a pulp containing about 55 to 65 per cent solids; simultaneously conditioning the resulting pulp with a sufficient amount of a material selected from the group consisting of water-soluble acids and acid salts yielding free acidic radicals in a solution to produce a pH of about 2.0 to 3.6 in the pulp, with an effective amount of an anionic promoter comprising a material selected from the group consisting of sulfonated oleic acid, sulfonated red oil, sulfonated methyl esters of red oil, and Turkey red oil, and with an effective amount of a cationic promoter comprising a mixture of hexadecyl, octadecyl, and octadecenyl amines; diluting the resulting conditioned pulp with water to a concentration of about 25 per cent solids; subjecting the resulting diluted pulp to froth flotation; and removing the resulting froth containing both micaceous materials and garnets.

9. A process for the production of ceramic-grade feldspar from a feldspathic ore containing iron both as micaceous materials and as garnets which comprises mixing such ore in a ground, deslimed state with water to form a pulp containing about 55 to 65 per cent solids; simultaneously conditioning the resulting pulp with a sufficient amount of a material selected from the group consisting of water-soluble acids and acid salts yielding free acidic radicals in

solution to produce a pH of about 2.0 to 3.1 in the pulp, with an effective amount of an anionic promoter comprising a material selected from the group consisting of sulfonated oleic acid, sulfonated red oil, sulfonated methyl esters of red oil, and Turkey red oil, and with an effective amount of a cationic promoter comprising a long-chain fatty-acid amine; diluting the resulting conditioned pulp with water to a concentration of about 25 per cent solids; subjecting the resulting diluted pulp to froth flotation; removing the resulting froth containing both micaceous materials and garnets; removing water from the resulting flotation tailing to a concentration of about 50 per cent solids; conditioning the resulting concentrated tailing with effective amounts of hydrofluoric acid, a long-chain fatty-acid amine, and a frothing agent; subjecting the conditioned tailing to froth flotation; and recovering ceramic-grade feldspar in froth as a flotation concentrate.

MASON K. BANKS.

#### REFERENCES CITED

25 The following references are of record in the file of this patent:

#### UNITED STATES PATENTS

| Number    | Name         | Date           |
|-----------|--------------|----------------|
| 2,132,902 | Lenher       | Oct. 11, 1938  |
| 2,297,689 | O'Meara      | Oct. 6, 1942   |
| 2,395,475 | Gibbs et al. | Feb. 26, 1946  |
| 2,483,192 | Gieseke      | Sept. 27, 1949 |
| 2,578,790 | Duke         | Dec. 18, 1951  |

#### FOREIGN PATENTS

| Number  | Country       | Date          |
|---------|---------------|---------------|
| 105,712 | Great Britain | Nov. 17, 1938 |

#### OTHER REFERENCES

40 Bulletin of American Ceramic Society, vol. 18, No. 8, August 1939, pages 286-292.